# EUROPEAN PATENT SPECIFICATION

(11) **EP 0 135 986 B1**
(45) Date of publication and mention of the grant of the patent: **09.09.1987**
(21) Application number: 84304384.5
(22) Date of filing: 28.06.1984
(51) Int. Cl.: B05D 1/26, B05D 7/14, B21D 22/20, C10M 111/04

(54) **Coated metal container and a method of forming such a container**
Beschichtete Metallbehälter und Verfahren zu seiner Formung
Récipient revêtu en métal et procédé pour sa formation

(30) Priority: 02.08.1983 US 519236
(43) Date of publication of application: 03.04.1985
(73) Proprietor: AMERICAN CAN COMPANY, Greenwich, Connecticut 06836-3610 (US)
(72) Inventor: Godar, Joseph L., Wauconda Illinois 60084 (US)
(74) Representative: Harvey, David Gareth

## Description

The present invention relates to a coated metal container and a method of forming such a container.

The well known three-piece sheet metal food or beverage container is fast being supplemented or supplanted by a two-piece container having a seamless body with one end wall integral with the body. A second end wall is secured to the body by means of a double seam after filling the container. Such containers for beer and soft drinks are made by the drawing and ironing process. Similar containers for fruits and vegetables require heavier and sturdier side walls and are beginning to be made by a newer process known as draw/ redraw.

Although the production of sheet metal containers by means of multiple draws is not new, the draw/redraw process is an improvement over the older drawing process in that it is done at higher speeds with greater draw ratios in each drawing step. Achieving this higher productivity rate requires special machines and, inter alia, special lubricants for the metal working operation.

To maintain this higher productivity rate, subsequent processing steps applied to the formed container must also be performed at high speed or eliminated where possible.

Butyl stearates have been used as rolling lubricants in steel mills and as lubricants for aiding in the mobility of synthetic fiber manufacture. Butyl stearate has been used for intricate metal forming operations such as bending tabs and necking and flanging can body ends, but has not been used for deep drawing. The need for butyl stearates in connection with particular precoating materials for can manufacture has not been appreciated.

The present invention involves the discovery that the butyl stearates not only act as effective lubricants in the drawing and redrawing of ferrous metal stock to form a container but that these lubricants when modified, unlike metal-working lubricants used heretofore, need not be removed from the surface of the formed container and may be used with vinyl based coatings without concern for the deterioration of same. Other lubricants useful as compatible postcoatable draw/ redraw lubricants have a plasticizing effect on the vinyl based coatings causing softening. In particular, an ATBC being a citric acid ester will soften a polyester or vinyl base coating when used therewith. The softened coating will scuff during the draw/redraw forming process. Coating damage is unacceptable since the coating must provide a complete barrier between the commestible and the metal container body.

One type of butyl stearate which works well is manufactured by C. P. Hall under their designation Uniflex Bys-Code C and has the following structural formula:

The method of the present invention has been found equally applicable for tinplated ferrous metal and for tin-free, low carbon sheet steel. The tinplate referred to in column 2, lines 50-56 of U.S.-A-4,287,741 is usable in the present invention, non-reflowed as well as matte finish tinplate described in U.S.-A-3,360,157. The tin weight on the steel basis metal may vary from 0.05 Ibs to 1.00 Ibs per base box (1.12 to 22.4 g . m-²). A base box comprises 31,360 sq in (202.3 cm²) of metal plate (the area being the area measured on one side).

According to FR-A-2,450,276, a coated metal container comprised a side wall and a bottom wall integral therewith, the side wall being of substantially the same thickness as the bottom wall or thinner and the metal of the said walls for example being electrolytic tinplate or tinless, low-carbon steel, the container walls being covered on at least the interior of the container, by a hardened coating of a synthetic resin applied atop a lanolin and silicone containing lubricant coating. Starting from this, the present invention provides such a container wherein the lubricant coating is a mixture consisting essentially of a butyl stearate, liquid lanolin and a silicone resin which mixture is compatible with the synthetic resin coating.

FR-A-2,450,276 also discloses a method of forming a coated metal container comprising the steps of applying a lanolin and silicone containing lubricant to a metal blank made for example of electrolytic tin plate or tinless, low carbon steel, drawing the blank by multiple draws to form a container, having integral side and bottom walls, applying a synthetic resin coating over at least the interior of the container and over the lubricant thereon, and heating the coated container to harden said synthetic resin coating. Such a method, according to the present invention, is characterised in that before drawing, the blank is coated with a lubricant mixture which consists essentially of a butyl stearate, liquid lanolin and a silicone resin, which mixture is compatible with said synthetic resin.

The preferred tin-free steel has a chromium surface treatment. While it is still in flat sheet form prior to its formation into a container, a synthetic resin base coat is applied and adhered to this treated surface. The most usual compositions for application as a base coat are those containing an epoxy resin, or vinyl resin, or polyester resin.

The invention will now be explained in more detail by way of example in the following non- limitative description.

The tin-free steel preferred for use in the present invention is aluminum killed, continuous cast steel with a chromium/chromium oxide surface treatment. The chromium in the oxide is present at about 0.5 to 2.0 mg per square foot (5.4 to 21.5 mg/m) and the chromium metal at about 3 to 13 mg per square foot (32.3 to 140 mg/m). The material described is known in the art as TFS-CT for tin-free steel, chromium type. The treatment is described in a paper published in the Journal of the Electrochemical Society, Vol., 116, No. 9, pp. 1299-1305.

The preferred tinplate has the same composition of steel as set forth above and at the steel mill in a well known manner, has tin applied to its surface electrolytically in various amounts, for example 0.25 Ib per base box (5.6 g . m-²). As mentioned, this tinplate may be left in a matte condition, i.e., is not flow brightened. The tinplate is oiled for rust inhibition and coiled for shipment to a container-making installation.

Thereafter, the tin-free steel when received in the can making plant has a base coating applied to its surfaces. The preferred coating contains a vinyl resin which is e.g. a vinyl organosol including low molecular weight vinyl copolymers, high molecular weight vinyl homopolymer dispersion resins and heat reactive cross linking resins to include phenolics, epoxies and aminoplasts. The preferred coating is manufactured by Midland Dexter of Waukegan, Illinois and is identified and sold as MM 519. This coating is known to contain as a primary resin a high molecular weight vinyl dispersion resin and lesser amounts of solution vinyl, polyester, epoxy and melamine resins as modifiers. While MM 519 performs well in the practice of this inyention there are situations when other coatings may be preferred. By way of example, another preferred coating is known to be MC 9788-101 sold by Mobil Chemicals. Unlike the MM 519, MC 9788-101 is not a vinyl organosol, and instead is composed of an isophthalic acid based polyester resin that is cured or cross-linked through the action of heat- reactive epoxy and melamine resins.

Those base coatings may be applied to both sides of the steel while the steel is still in coil form or the steel may be cut into scrolled sheets and the coating applied to individual sheets, which coating is subsequently baked to form a tough, adherent base coat on the tin-free steel.

The butyl stearate lubricant mixture of the present invention is either electrostatically coated, dip coated or spray coated onto both surfaces of individual sheets of the base coated tin-free steel. The sheets are then fed into a blanking and cupping press which cuts from the sheet one or more circular discs of 7.947 in (20.18 cm) in diameter, and draws the disc into a cup of 5.007 in (12.72 cm) in diameter and 1.850 inches (4.69 cm) in side wall height. In two subsequent operations, the cup is successively reduced in diameter with concurrent lengthening of its side wall, i.e., drawn; and simultaneously the side wall is slightly thinned, i.e. to about 10% less than the starting gauge, and further elongated, i.e., ironed, in the manner similar to that described in U.S.-A-3,360,157. The final diameter and side wall height accomplished in the drawing plus ironing are 3.060 in and 4.450 in (7.77 and 11.30 cm) respectively and are accomplished in a few seconds. The diameter of the starting blank, the height-to-diameter ratios, and the draw ratios, in the ensuing metal working process may be varied depending upon the desired size of the finished can. Also, as between different draw/redraw systems, the amount of draw in each step may be varied providing the cumulative effect of the plural draws and with ironing produces the can of desired height and diameter.

The severity of the concurrent diameter reduction and side wall thinning (ironing) requires an excellent lubricant which will not attack the coating. It is readily apparent that a draw/redraw system with ironing is a more severe metal working process than a draw/redraw system without ironing. The butyl stearate lubricant of the present invention performs equally well in both systems.

The amount of lubricant applied over the base coat can vary from 10 to 40 mg/sq ft (108 to 431 mg - m-²) and preferably 10 to 20 mg/sq ft (108 to 215 mg - m-²) of total surface, i.e., both sides, of the sheet being fed into the draw/redraw apparatus. It has been found that the lubricating effect falls off appreciably below 10 mgs/ft² (108 mg m-2) and for most operations 20 mgs/ft² (215 mg . m-2) is sufficient to achieve the high speed, trouble free, multiple draws from flat blank to formed container. Susbtantial heat is generated on the surfaces being worked due to the severity of the metal-working operation, i.e., the appreciable draw ratios and draw speed plus ironing.

No particular theory is known as to why the butyl stearate lubricant is compatible for postcoating without need for removal of same. Other lubricating materials (under identical conditions) have been known to attack the base coating as already described. Moreover, the severe metal forming operations of precoated sheet at high speed and pressure would drive the lubricant into the coating and so a lubricant which is compatible with the coating even under such conditions is needed.

Certain silicone resins such as General Electric's SR 82 are known for their ability to modify coatings and thereby enhance their bond with a metal substrate to which they are applied. However, the addition of silicon resin such as General Electric's SR 82 to butyl stearate to permit subsequently applied coatings (after forming) to cover the surface of the metal substrate completely was not appreciated. That is to say, the addition of silicone resin to the butyl stearate allows complete coverage of all portions of metal substrates by coatings applied after forming without leaving eye holes or discontinuities in the coverage and without any tendencies for the postcoating to bead up. The effect without silicone resin is much like water on freshly waxed surfaces. The addition of silicone resin permits a wetting action and alters the surface tension of the butyl stearate sufficiently to allow the coatings as applied to spread evenly and completely over the lubricated metal substrate and to form a good bond over the entire surface. The proposed combination of silicone resin and butyl stearate when preapplied to coils or panels of tin free steel plate, electrolytic tinplate or other materials for deep drawing containers or cup-like objects which are intended to be post sprayed or post decorated performs successfully because of the bonding and good adherence of the wettable combination to the lubricated metal surface.

### Compatibility lube-Wettability test

Ingredients which have good lubricating properties were tested for compatibility with the postsprayed top coat.

The test procedure consisted of wiping a thin film of the lubricant on a piece of base coated plate (the lubricant was applied at a weight of about 50 to 75 mgs sq ft-538 to 807 mg . m-²). A water base top coating was then sprayed over the lubricant bearing plate. These panels were allowed to stay at room temperature for at least 15 minutes to see if the coating would de-wet from the lubricant treated area.

The results with the various lubricants tried were as follows:
1. Butyl stearate-no de-wetting.
2. Liquid lanolin-very slight de-wetting.
3. SR-882 silicone-no de-wetting.
4. Petrolatum-severe de-wetting.

Using this test procedure combinations of the lubricants listed were tried and when these ingredients are blended at the proper ratios (not petrolatum) no de-wetting of the spray top coat occurred.

For sheet feeding, the lubricant mixture must have less than 50% liquid lanolin. Adjacent sheets stick together when the lanolin is applied at heavier rates. For coil stock or prelube spot coating the liquid lanolin level may be increased beyond the 50%.

### Discussion of the various lubricants

While butyl stearate is a lubricant it is really inadequate for the heavy loads in draw and redraw forming operations. Enhanced lubricity can be had by the addition of liquid lanolin but use of lanolin, without reduction of its viscosity, with butyl stearate makes difficult application at the mentioned rates. The use of butyl stearate only will not be adequate to lubricate the material as the latter is drawn and redrawn. Conversely, the use of liquid lanolin only would be a problem because of its viscosity. Therefore, the combination of butyl stearate and liquid lanolin are important.

There may also be a need for something which will allow the combination to be postcoated. If lubrication were the only requirement and a complete coverage of the metal surface were not necessary, the drawing tools might tend to spread whatever lubricant is available. The postcoating of lubricant could be effected by the build-up of the lube on the tools. That is, the lube would be sufficient to lubricate for the forming process but the material might be slightly over lubricated in certain areas. The additional wetting provided by General Electric's SR 82 silicone resin is necessary to provide sufficient wettability to the metallic substrate for the postcoating.

Drawing and redrawing are not the only forming operations the lubricated container must endure. At the completion of the draw/redraw operation, the container is beaded to impart strength to the side and bottom walls before being fed into a device for applying a top coat to the container's inside surface. Most usually, this device involves a turret which revolves the container past a reciprocating spray gun which enters the interior of the container as same is spun about its longitudinal axis. The spray gun is retracted from the container body and emits a 360° spray of a synthetic resin solution to coat the entire interior surface of the container.

After completion of the top coating operation, the container is then subjected to a temperature of 400°F (204°C) for 2 to 4 minutes to harden and cure the top coat. Unlike prior procedures of metal forming which required the formed metal container to be washed to remove lubricant and then dried before application of the top coat, thereby to avoid contamination and improper curing of the top coat, the procedure of the present invention not only eliminates the expense and time-consuming step of removing the lubricant but also permits the application of the top coat directly to a still lubricated surface (the inside of the container). In addition, the wetted lubricant remaining after forming assists in firmly adhering the top coat to the base coat.

The butyl stearate and what remains thereof after the draw/redraw operation are soluble in organic solvents such as butanol, butyl Cellosolve, diisobutyl ketone, Cellosolve acetate and Solvesso 150. Therefore, resins for top coats which are also soluble in these same solvents and provide inert, continuous, resin films upon thermal curing are preferred. More particularly, resins such as epoxy resins, acrylic resins and vinyl resins are useful and particularly usable if they are applied over a vinyl base coat and a lubricant which does not attack the vinyl or cause softening.

Evaluation of top coats applied over a butyl stearate lubricated vinyl base coat is done by testing process resistance as well as examination of intercoat adhesion between the base coat and the top coat. Intercoat adhesion is tested with a pressure sensitive adhesive tape. More particularly, a one inch strip (2.54 cm wide) of "3M" tape #610 is applied to the surface of the top coated sample. The tape is pressed to the surface with sufficient pressure to make complete contact (removing the air bubbles therebetween). The tape test requires that the tape be quickly pulled from the sample in an effort to peel with it any poorly adhering coating. In order to further test peeling, X's are scribed on the surface across which the tape is to be applied. These X's present freshly made scored edges which would help to initiate any peeling that might occur. Examples 1 to 5 which follow herein were tested for intercoat adhesion by this method and all passed. No separation of the top coat from the compatably lubricated base coat occurred.

Similarly, the continuity of the top coat can be tested by the quick test method. In order to perform a quick test a specific piece of equipment is required. More particularly, a Model 1071 WACO Enamel Rater with a 0 to 1 milliamp attachment is used. The apparatus has an electrode which is adapted to move vertically in and out along the axis of a can positioned beneath it. The electrode is positioned about 1" (2.5 cm) from the bottom of the can. The can is held in position by a vice-like device which clamps it about the bottom holding it so that the open end of the can faces up toward the electrode. The can is filled with 2% solution of sodium sulfate and allowed to soak for at least 30 seconds before the electrode is dropped into the can. The solution temperature should be maintained between 72 to 78°F (22 to 25.5°C), and the can should be filled so that when the electrode is lowered into the test position the solution will reach approximately 1/8" (3 mm) below the top flange radius of the can. Care should be taken to avoid wetting the flange since that will result in a false high reading. The milliamp meter of the tester is connected to the vice-like device which holds the bottom of the can. The electrode is connected to another lead of the milliamp meter. A zeroing of the instrument is required and the operator adjusts the milliamp to read "T" on the scale. Shortly after zeroing the meter a warning light comes on and the reading should be taken immediately. When this procedure is applied to properly coated cans readings in the range of 0 to 5 milliamps should be obtained and such data is indicative of an acceptable container.

Consequently, a coating system for a metal substrate which will withstand the severity of multiple forming operations without destruction has been sought. A coating system which functions to protect the metal substrate and prevent corrosion and off flavor is the thrust of this invention.

### Example 1

A composition designated Formula 29-1 including 40% liquid lanolin made by Kraft and designated Ritalan was mixed with 50% n-butyl stearate made by C. P. Hall and 10% silicone resin with an abundance of hydroxyls made by General Electric and called SR-82 were mixed together and applied to tin free steel designated TFS-CT which was base coated with 33 mg per 4 square inches (1.28 mg . cm-²) of a vinyl coating made by Midland-Dexter and designated MM-519. The base coating was cured at 400°F (204°C) for 8 minutes. The composition of Formula 29-1 was applied at a rate of 25 mg per square foot (269 mg . m-²) by means of spray.

These samples were tested as follows. The scroll strips did not stick to one another with this formula. Thus, there was adequate viscosity reduction of the lanolin. They feed well and make excellent cans when drawn and redrawn and can be postsprayed over directly without first washing and drying.

### Example 2

A composition designated Formula 28-1 including 55.55% liquid lanolin made by Kraft and designated Ritalan was mixed with 26.67% n-butyl stearate made by C. P. Hall and 17.78% silicone resin with an abundance of hydroxyls made by General Electric and commercially available as SR-82 were mixed together and applied to tin free steel designated TFS-CT which was base coated with 33 mg per 4 square inches (1.28 mg . cm-²) of a vinyl coating made by Midland Dexter and designated MM-519. The base coating was cured at 400°F (204°C) for 8 minutes. The composition of Formula 28-1 was applied at a rate of 25 mg per square foot (269 mg . m-²) by means of spray.

These samples were tested and this formula caused the scroll strips to stick slightly, hampering feeding, because the lanolin was still too viscous. Good cans were made.

### Example 3

A composition designated Formula 26-4 including 66% liquid lanolin made by Kraft and designated ritalan was mixed with 27% n-butyl stearate made by C. P. Hall and 17% silicone resin with an abundance of hydroxyls made by General Electric and called SR-82 were mixed together and applied to tin free steel designated TFS-CT which was base coated with 33 mg per 4 square inches (1.28 mg . cm-²) of a vinyl coating made by Midland Dexter and desigriated MM-519. The base coating was cured at 400°F (204°C) for 8 minutes. The composition of Formula 26-4 was applied at a rate of 25 mg per square foot (269 ₘg . m-²) by means of spray.

These samples were tested and this formula did not allow the scroll strips to feed into the press. The high lanolin content made the composition viscous causing the strips to stick together. The lube allowed the cans to form very well.

### Example 4

A composition designated Formula 29-1 including 40% liquid lanolin made by Kraft and designated Ritalan was mixed with 50% n-butyl stearate made by C. P. Hall and 10% silicone resin with an abundance of hydroxyls made by General Electric and called SR-82 were mixed together and applied to tin free steel designated TFS-CT which was base coated with 33 mg per 4 square inches (1.28 mg - cm-²) of a polyester coating made by Mobil and designated MC-9788-101. The base coating was cured at 400°F (204°C) for 8 minutes. The composition of Formula 29-1 was applied at a rate of 25 mg per square foot (269 ₘg . m-²) by means of spray.

The samples were tested and excellent cans were made, with no problems of scroll strips sticking together and with good postspray coverage.

### Example 5

A composition designated Formula 24-10 including 17.17% liquid lanolin made by Kraft and designated Ritalan, 66.99% n-butyl stearate made by C. P. Hall, and 15.84% silicone resin with an abundance of hydroxyls made by General Electric and called SR-82 were mixed together and applied to tinplated steel designated #25 ETP, which was electrolytically coated steel having 0.25 pounds of tin coating per base box (5.6 g . m-²). Sample containers were then made from this plate using three draw/redraw steps. The completed cans were then inside post sprayed without removing the residual lubricant after the drawing operations. The spray coating used was an aliphatic hydrocarbon, solvent-based aluminium pigmented modified epoxy phenolic resin. The post coating was cured at 400°F (204°C) for 5-1/2 minutes. The composition of Formula 24-10 was applied at a rate of 20 mg per square foot (215 mg - m-²) by means of a dip tank and squeegee metering. There were no fabrication failures during a 2000 can run using plate lubricated with this formula.

The sample containers of Examples 1, 4 and 5 were evaluated by means of a quick test procedure commonly used by can makers to determine the degree of coverage of inside sprayed containers. Quick test readings of zero are desirable, but values up to 5 milliamperes of current flow during the testing procedure are usually considered good. The sample containers tested had a quick test range of 0 to 5, with the average being about 1.5 milliamperes.

A typical container as formed by the draw/ redraw process using the lubricant combination of this invention results in a 303x406 two-piece tin plated steel can. A 303x406 can is one having a diameter of 3-3/16 in and a height of 4-3/8 in (81 x 111 mm approximately). The inside diameter of the triple drawn finished container of examples is 3.060" (77.7 mm), the height is 4.375" (111.1 mm), and the bottom and sidewall thickness are approximately .0083" (0.21 mm), when the feed stock was 75 #T-4 plate. Tin plate, either TFS-CT tin free steel or electrolytic tinplate having various tin weights deposited on both sides of the plate will perform acceptably.

While the preceding description has dealt with various examples and various materials, the invention in its broadest aspect is considered to include any type of silicone resin with liquid lanolin (the viscosity of which is reduced by the butyl stearate) to permit a subsequently applied organic coating to spread evenly over the remaining combination after a deep drawing operation resulting in a good bond to the metal substrate after curing of the coating. For specific applications which require more severe draws and/or thinner post coatings, the amounts of the various constituents in the combination can be varied in order to maintain low costs with a lubricant which will perform successfully. In addition, post coating of all ranges of tin coverage on steel will work successfully with this type of lubricant combination. Lightly precoated tin free steels (TFS-CT) can also be successfully processed into post coated containers in accordance with this invention.

## Claims

1. A coated metal container comprising a side wall and a bottom wall integral therewith, the side wall being of substantially the same thickness as the bottom wall or thinner and the metal of the side walls for example being electrolytic tinplate or tinless, low-carbon steel, the container walls being covered on at least the interior of the container, by a hardened coating of a synthetic resin applied atop a lanolin and silicone containing lubricant coating, characterised in that the lubricant coating is a mixture consisting essentially of a butyl stearate, liquid lanolin and a silicone resin which mixture is compatible with the synthetic resin coating.

2-The metal container according to claim 1, wherein the synthetic resin coating is selected from polyester, acrylic and vinyl resins.

3. The metal container according to claim 1 or claim 2, wherein a hardened synthetic resin base coat is interposed between the walls and the said hardened coating, the base coat covering and adhering to said walls, and the base coat being a resin selected from polyester, vinyl, epoxy and acrylic resins.

4. The metal container according to claim 1, 2 or 3, wherein the metal is non-reflowed, matte finish tinplate or tin-free steel with a chromium treated surface.

5. The metal container according to any of claims 1 to 4, wherein the lubricant coating contains less than 50% by weight of lanolin.

6. The metal container according to claim 5, wherein the lubricant coating contains 40% liquid lanolin, 50% n-butyl stearate and 10% silicone resin.

7. The metal container according to claim 5, wherein the lubricant coating contains about 17% liquid lanolin, about 67% n-butyl stearate and about 16% silicone resin.

8. A method of forming a coated metal container comprising the steps of applying a lanolin and silicone containing lubricant to a metal blank made for example of electrolytic tin plate or tinless, low carbon steel, drawing the blank by multiple draws to form a container, having integral side and bottom walls, applying a synthetic resin coating over at least the interior of the container and over the lubricant thereon, and heating the coated container to harden said synthetic resin coating, characterised in that before drawing, the blank is coated with a lubricant mixture which consists essentially of a butyl stearate, liquid lanolin and a silicone resin, which mixture is compatible with said synthetic resin.

9. The method according to claim 8, wherein the side wall of said cup is subjected to ironing during the multiple draws whereby the side wall of said container is made thinner than the bottom wall.

10. The method according to claim 8 or claim 9, wherein a base coating is applied to and adhered to the metal prior to the application of said butyl stearate/lanolin/silicone resin mixture, the base coating being selected from polyester, vinyl and acrylic resins.

11. The method according to claim 8, 9 or 10, wherein the lubricant mixture contains 40% liquid lanolin, 50% n-butyl stearate and 10% silicone resin.

12. The method according to claim 8, 9 or 10, wherein the lubricant mixture contains about 17% liquid lanolin, about 67% n-butyl stearate and about 16% silicone resin.

13. The method according to any of claims 8 to 12, wherein the synthetic resin is selected from polyester, vinyl and acrylic resins.

14. The method according to any of claims 8 to 13, wherein the lubricant mixture is applied to the blank at a coverage rate of 10 to 40 mg/sq ft (108 to 431 mg - m-²) of total surface.

## Patentansprüche

1. Beschichteter Metallbehälter, betehend aus einer Seitenwand und einer mit dieser einstückigen Bodenwand, wobei die Seitenwand von im wesentlichen der gleichen Dicke wie die Bodenwand oder dünner ist und das Metall der Seitenwände zum Beispiel ein elektrolytisch verzinntes Weißblech oder oder ein zinnfreier, niedriggekohlter Stahl ist und die Behälterwände zumindest auf der innenseite des Behälters von einer gehärteten Beschichtung eines Kunstharzes bedeckt sind, die oben auf eine Lanolin und Silikon enthaltende Schmiermittelbesrchichtung aufgebracht ist, dadurch gekennzeichnet, daß die Schmiermittelbeschichtung ein Gemisch ist, das im wesentlichen aus einem Butylstearat, flüssigem Lanolin und einem Silikonharz besteht, welches Gemisch mit der Kunstharzbeschichtung verträglich ist.

2. Metallbehälter nach Anspruch 1, dadurch gekennzeichnet, daß die Kunstharzbeschichtung aus Polyester-, Akryl- und Vinylharzen ausgewählt ist.

3. Metallbehälter nach Anspruch 1 oder 2, dadurch gekennzeichnet, daß eine gehärtete Kunstharzbasisschicht zwischen den Wänden und der gehärteten Beschichtung angeordnet ist, die die Wände bedeckt und an ihnen anhaftet, und daß die Basisschicht aus einem aus Polyester-, Vinyl-, Epoxid- und Akrylharzen ausgewählten Harz besteht.

4. Metallbehälter nach Anspruch 1, 2 oder 3, dadurch gekennzeichnet, daß das Metall ein nicht-zurückgeschmolzenes, mattes Weißblech oder ein zinnfreier Stahl mit einer chrombehandelten Oberfläche ist.

5. Metallbehälter nach einem der Ansprüche 1 bis 4, dadurch gekennzeichnet, daß die Schmiermittelbeschichtung weniger als 50 Gew.-% Lanolin enthält.

6. Metallbehälter nach Anspruch 5, dadurch gekennzeichnet, daß die Schmiermittelbeschichtung 40% flüssiges Lanolin, 50% n-Butylstearat und 10% Silikonharz enthält.

7. Metallbehälter nach Anspruch 5, dadurch gekennzeichnet, daß die Schmiermittelbeschichtung etwa 17% flüssiges Lanolin, etwa 67% n-Butylstearat und etwa 16% Silikonharz enthält.

8. Verfahren zur Formung eines beschichteten Metallbehälters, bei dem ein Lanolin und Silikon enthaltendes Schmiermittel auf einen zum Beispiel von einem elektrolytisch verzinnten Weißblech oder einem zinnfreien, niedriggekohlten Stahl gebildeten Metallrohling aufgebracht, der Rohling durch mehrfache Ziehvorgänge zur Formung eines Behälters mit einstückigen Seiten-und Bodenwänden gezogen, eine Kunstharzbeschichtung auf zumindest der Innenseite des Behälters und über dem darauf befindlichen Schmiermittel aufgebracht und der beschichtete Behälter zum Härten de Kunstharzbeschichtung erwärmt wird, dadurch gekennzeichnet, daß vor dem Ziehvorgang der Rohling mit einem Schmiermittelgemisch beschichtet wird, das im wesentlichen aus einem Butylstearat, flüssigem Lanolin und einem Silikonharz besteht, welches Gemisch mit dem Kunstharz verträglich ist.

9. Verfahren nach Anspruch 8, dadurch gekennzeichnet, daß die Wand des Behälters während der Mehrfachziehvorgänge einem Abstreckvorgang unterzogen wird, wodurch die Seitenwand des Behälters dünner als die Bodenwand ausgebildet wird.

10. Verfahren nach Anspruch 8 oder 9, dadurch gekennzeichnet, daß eine Basisbeschichtung auf das Metall vor der Aufbringung des Butylstearat/ Lanolin/Silikonharz-Gemisches, aufgetragen und zum Anhaften gebracht wird, wobei die Basisbeschichtung aus Polyester-, Vinyl- und Akrylharzen ausgewählt wird.

11. Verfahren nach Anspruch 8, 9 oder 10, dadurch gekennzeichnet, daß das Schmiermittelgemisch 40% flüssiges Lanolin, 50% n-Butylstearat und 10% Silikonharz enthält.

12. Verfahren nach Anspruch 8, 9 oder 10, dadurch gekennzeichnet, daß das Schmiermittelgemisch etwa 17% flüssiges Lanolin, etwa 67% n-Butylstearat und etwa 16% Silikonharz enthält.

13. Verfahren nach einem der Ansprüche 8 bis 12, dadurch gekennzeichnet, daß das Kunstharz aus Polyester-, Vinyl- und Akrylharzen ausgewählt wird.

14. Verfahren nach einem der Ansprüche 8 bis 13, dadurch gekennzeichnet, daß das Schmiermittelgemisch auf den Rohling mit einer Bedekkungsrate von 10 bis 40 mg/Quadratfuß (108 bis 431 mg m-²) der Gesamtoberfläche aufgebracht wird.

## Revendications

1. Récipient révêtu en métal comprenant une paroi latérale et une paroi de fond formant une partie intégrante de ladite paroi latérale, ladite paroi latérale ayant substantiellement la même épaisseur que la paroi de fond ou étant plus mince que celle-ci et le métal des parois latérales étant par exemple du fer blanc électrolytique ou de l'acier à faible teneur en carbone sans étain, les parois du récipient étant recouvertes au moins sur l'intérieur du récipient d'un revêtement durci d'une résine synthétique appliquée sur un revête- . ment lubrifiant contenant de la lanoline ou de la silicone, caractérisé en ce que le revêtement lubrifiant est un mélange composé essentiellement de stéarate de butyle, de lanoline liquide et d'une résine de silicone, ledit mélange étant compatible avec le revêtement en résine synthétique.

2. Récipient en métal selon la revendication 1, dans lequel le revêtement en résine synthétique est choisi des résines polyester, acrylique et vinylique.

3. Récipient en métal selon la revendication 1 ou 2, dans lequel un revêtement de base en résine synthétique durcie est interposé entre les parois et ledit revêtement durci, le revêtement de base recouvrant et adhérant auxdites parois, et le revêtement de base étant une résine choisie des résines polyester, vinylique, epoxy et acrylique.

4. Récipient en métal selon la revendication 1, 2 ou 3, dans laquelle le métal est du fer blanc non refondu à finition mate ou de l'acier sans étain ayant une surface traitée au chrome.

5. Récipient en métal selon l'une quelconque des revendications 1 à 4, dans lequel le revêtement lubrifiant contient moins de 50% en poids de lanoline.

6. Récipient en métal selon la revendication 5, dans lequel le revêtement lubrifiant contient 40% de lanoline liquide, 50% de stéarate de n-butyle et 10% de résine de silicone.

7. Récipient en métal selon la revendication 5, dans lequel le revêtement lubrifiant contient environ 17% de lanoline liquide, environ 67% de stéarate de n-butyle et environ 16% de résine de silicone.

8. Procédé pour former un récipient en métal revêtu comprenant les étapes d'appliquer un lubrifiant contenant de la lanoline et de la silicone sur une ébauche métallique fait par exemple de fer blanc électrolytique ou d'acier à faible teneur en carbone sans étain, étirer l'ébauche en plusieurs étapes pour former un récipient ayant des partois intégrales latérale et de fond, appliquer un revêtement en résine synthétique au moins sur l'intérieur du récipient et sur le lubrifiant qui s'y trouve et chauffer le récipient revêtu pour durcir le revêtement en résine synthétique, caractérisé qu'avant l'étirage l'ébauche est revêtue d'un mélange lubrifiant qui consiste essentiellement en stéarate de butyle, de la lanoline liquide et de la résine de silicone, ledit mélange étant compatible avec ladite résine synthétique.

9. Procédé selon la revendication 8, dans lequel la paroi latérale de ladite coupe est soumise à l'étirage pendant les multiples étapes de sorte que la paroi latérale du récipient devient plus mince que la paroi de fond.

10. Procédé selon la revendication 8 ou 9, dans lequel un revêtement de base est appliqué et adhère au métal avant l'application dudit mélange de stéarate de butyle/lanoline/résine de silicone, ledit revêtement de base étant choisi des résines polyester, vinylique et acrylique.

11. Procédé selon la revendication 8, 9 ou 10, dans lequel le mélange lubrifiant contient 40% de lanoline liquide, 50% de stéarate n-butyle et 10% de résine de silicone.

12. Procédé selon la revendication 8, 9 ou 10 dans lequel le mélange lubrifiant contient environ 17% de lanoline liquide, environ 67% de stéarate n-butyle et environ 16% de résine de silicone.

13. Procédé selon l'une quelconque des revendications 6 à 12, dans lequel la résine synthétique est choisie des résines polyester, vinylique et acrylique.

14. Procédé selon l'une quelconque des revendications 8 à 13, dans lequel le mélange lubrifiant est appliqué à l'ébauche à une vitesse de recouvrement de 10 à 40 mg/pd² (108 à 431 mg/m²) de surface totale.
